# EUROPEAN PATENT SPECIFICATION

(11) **EP 0 025 279 B1**
(45) Date of publication and mention of the grant of the patent: **14.03.1984**
(21) Application number: 80302760.6
(22) Date of filing: 12.08.1980
(51) Int. Cl.: C10L 1/32

(54) **A method for the preparation of a uniform solid fuel-oil dispersion**
Verfahren zur Herstellung einer gleichmässigen Dispersion eines festen Brennstoffs in Öl
Procédé de préparation d'une dispersion uniforme d'un solide combustible dans une huile

(30) Priority: 15.08.1979 GB 7928409
(43) Date of publication of application: 18.03.1981
(73) Proprietor: The British Petroleum Company p.l.c., London EC2Y 9BU (GB)
(72) Inventor: Veal, Christopher John, Sunbury-on-Thames Middlesex, TW16 7LN (GB); Wall, Derek Richard, Sunbury-on Thames Middlesex, TW16 7LN (GB)
(74) Representative: MacLeod, Malcolm

## Description

This invention relates to the preparation of dispersion of solid fuels in liquid fuels in tumbling ball mills and, more particularly, to the preparation of dispersions of coal in oil.

Our British Patent Specification No. 1523193 discloses a method for the preparation of coal oil dispersions which method comprises grinding coal in a medium consisting essentially of gas oil and/or a heavier petroleum fraction until the particle size is reduced to a value below 10 ,um and the dispersion contains 15 to 55% by weight coal expressed as a percentage by weight of the total dispersion. 1523193 discloses that grinding can be carried out in vibratory or agitatory ball mills.

Tumbling ball mills are, of course, well known grinding machines and have been used in the past in both batch and continuous processes. They have been used primarily for the dry grinding of friable solids such as cement clinker. In certain applications, however, it is desirable to grind in the wet state, that is, when the solids are suspended in a liquid forming a slurry. The liquid concerned is normally water. An example of such a process is the beneficiation of metal bearing ores. In some cases, e.g. paint manufacture and metal powder processing, light hydrocarbon fractions are employed. The latter tend to be batch processes, however, carried out on a small scale.

Journal Soc. Chem. Ind. Vol. 39, 1920, p. 395 discloses that "colloidal fuel" may be prepared by grinding coal in oil in tube mills. The term "colloidal fuel" was used loosely at that time to describe relatively coarse suspension of coal in oil The most relevant fuel described contained coal particles ground so that at least 90% passed through a 100 mesh screen (B.S.S.) and 85% through a 200 mesh screen (B.S.S.). Such dimensions are far in excess of colloidal dimensions quoted by Glasstone as being in the range 0.2-0.005 ,um. (Glasstone, Textbook of Physical Chemistry; Second Edition, Macmillan & Co. Ltd., London, 1953, page 1232.

It was, in fact, believed that a tumbling ball mill would be incapable of wet milling solid particles such as coal to an average particle size of 10 µm or less, in the presence of a grinding medium such as fuel oil.

We have now surprisingly discovered that a tumbling ball mill can be used in the preparation of such fine dispersions.

Thus according to the present invention there is provided a method for the preparation of a uniform solid fuel-oil dispersion which method comprises grinding the solid fuel in a fuel oil medium until-the mean solid particle size is reduced to a value in the range 1 to 10 µm, preferably 2 to 5 µm, and the dispersion contains 15 to 55% by weight solid fuel, preferably 30 to 45%, expressed as a percentage by weight of the total dispersion characterised in that grinding takes place on a tumbling ball mill.

Suitable friable solids include coals of various ranks, solvent refined coal, coal coke and petroleum coke. The preferable friable solid is bituminous coal.

A suitable oil is a petroleum fuel oil fraction having a viscosity of not more than 1500 mm²/sec (600 seconds, Redwood No 1), preferably not more than 850 mm²/sec (3500 seconds, Redwood No 1) at 100°F (37.8°C). The required viscosity may be achieved by "cutting back" if necessary with, for example, gas oil.

In the case of certain heavier fuel oil fractions it may be necessary to heat them in order to render them sufficiently mobile to permit use as a grinding liquid, initially in the case of a batch process or at the entry to the mill in the case of a continuous process. However, the action of grinding generates a considerable quantity of heat.

The tumbling ball mill is preferably operated under standard tumbling ball mill conditions, i.e. with the balls occupying 10-50%, most preferably 30-45%, of the internal volume, with the mixture of solid fuel and oil occupying 5 to 45%, and the speed of rotation of the mill about 60 to 95%, preferably 70 to 80%, of the critical speed which is defined as the lowest speed at which a single element of the charge would be held against the internal surface by centrifugal force.

Under these conditions with a viscous grinding liquid the contents of a tumbling ball mill will take up a kidney shaped configuration as the mill rotates. This cascades smoothly with little splashing or surging. Grinding takes place mostly in the interior of the kidney shaped mass and freshly ground surfaces are exposed to the gaseous atmosphere in the mill to a lesser extent than they would be in partially filled vibratory or agitatory ball mills, thus excluding the atmosphere from a substantial proportion of the grinding activity.

If no special precautions are taken, this atmosphere will normally be air. However, in order to reduce the risk of free oxygen contamination still further, in view of the adverse effect which this has on product stability, it is preferred to operate the tumbling ball mill with the contents under an inert blanket, e.g. of nitrogen. This has the further advantage of eliminating the risk of forming hazardous vapour mixtures. Inert gas blanketing is particularly advantageous when grinding at relatively high temperatures, e.g. close to or above the flash point of the oil.

Preferably the solid fuel supplied to the tumbling ball mill is preground to a particle size not greater than 250,um. This may be achieved by conventional size reducing machinery such as attritors, hammer mills, etc.

Alternatively, lump coal can be supplied to the ball mill and ground down to its final size within the mill.

It is not necessary to premix the preground solid fuel with the oil since the tumbling ball mill acts as a mixer as well as a grinder.

When using a large tumbling ball mill often known as a tube mill, e.g., having a length to diameter ratio of greater than 3:1, it may be desirable to subdivide the mill into a number of compartments separated by screens through which the mixture can flow. In order to achieve more efficient grinding, the size of the balls is progressively reduced from the inlet chamber to the outlet chamber.

It is, of course, desirable to use balls made of a material which does not react with the solid fuel and the oil and which does not wear unduly either itself or the interior surface of the mill. Ball mills usually contain steel balls and these are suitable for the present purpose.

The dispersions will generally be prepared, used and stored at elevated temperature and under these conditions will be more stable than corresponding dispersions prepared in the presence of air.

The solid fuel-oil dispersions are suitable for use in blast furnaces, cement kilns and in industrial, marine and utility boilers.

The stability of the solid fuel-oil dispersion is a function of three important variables-the method of grinding, the final particle size and the concentration of solid in oil. If all three are chosen correctly then the dispersion is of enhanced stability at elevated and ambient temperatures.

At ambient temperature, the dispersion is in the form of a weak, thixotropic gel in which a physical network is formed by solid particles in oil. It is a uniform structure from which the solid particles cannot settle out because they form part of it. This is unlike coal oil dispersions prior to those disclosed in 1523193 which were merely slurries in which the coal particles were suspended in the oil from which they would eventually settle out or colloidal suspensions.

At elevated temperature, although the gel- like structure is less apparent, the same interactions occur to confer enhanced stability.

If the solid particles are not ground in the oil in the absence of air, the solid particles will become oxidised and interact unfavorably. If the solid particle size is too great, forces will be insufficient to confer stability. The concentration of the solid particles is also critical. If it is too low, the dispersion will be unstable. If it is too high, the dispersion will become too solid like for pumping.

The invention is illustrated with reference to the accompanying drawing, which is a block diagram of a method for producing a coal-oil dispersion according to the present invention, and the Example.

With reference to the drawing:
Lump coal is supplied by line 1 to a screen 2 which passes lumps of size below 6.4 mm to an attritor 3 which reduces the particle size to 70% wt below 200 mesh. Oversize lumps from the screen 2 are reduced in size in a jaw-crusher 4 and returned to the screen 2. Particles from the attritor 3 move to a classifier 5 from which particles below 212 ,um in size are passed by an air lift to storage 6 and oversize particles are returned to the attritor 3 for further comminution.

Oil is supplied by line 7, passed through a heater 8 and powdered coal from storage 6 is added to the oil at the entry to a tumbling ball mill 9. The mill is divided into three chambers separated by screens 10 and 11. The mill supplied with nitrogen by means (not shown) to provide an inert atmosphere within the mill.

The coal-oil mixture passes continuously through the chambers of the mill and is removed by line 12.

### Example

The coal was Pleasley Washed Singles with the following ultimate and initial particle size analysis (as received).

The oil was a mixed source heavy fuel oil with a viscosity of 50 mm²/s (3500 seconds Redwood No 1) at 100°F (37.8°C). It had the following properties:

The coal was passed through the pre- grinding system described with reference to the drawing and passed to storage 6, with a maximum particle size of 212 ,um.

The oil from storage at 80°C was passed through the heater 8 where its temperature was raised to 120°C.

Near the entry to the mill 9 which was approximately 2 m diameter and 10m long coal was added to the oil to give a mixture containing 40% by wt coal. This material was then ground in the mill which was loaded to about 40% volume with steel balls.

The mill was operated at a speed of 24 rpm (80% critical).

Nitrogen was supplied to the interior of the mill and cooling water to the mill bearings.

The mean particle size of the coal after grinding was 3.7 um as determined by an optical microscope technique.

A sample of the dispersion prepared above showed no signs of settling after standing for 24 hours at 100°C.

## Claims

1. A method for the preparation of a uniform solid fuel-oil dispersion which method comprises grinding the solid fuel in a fuel oil medium until the mean solid particle size is reduced to a value in the range 1 to 10 µm and the dispersion contains 15 to 55% by weight solid fuel expressed as a percentage by weight of the total dispersion, characterised in that grinding takes place in a tumbling ball mill.

2. A method according to claim 1 wherein the mean particle size of the solid fuel is reduced to a value in the range 2 to 5 ,um.

3. A method according to either of the preceding claims wherein the dispersion contains 30 to 45% by weight solid fuel expressed as a percentage by weight of the total dispersion.

4. A method according to any of the preceding claims wherein the friable solid is coal, solvent refined coal, coal coke or petroleum coke.

5. A method according to claim 4 wherein the friable solid is bituminous coal.

6. A method according to a: of the preceding claims wherein the solid fuel is preground to a particle size not greater than 250,um before grinding in the oil medium.

7. A method according to any of the preceding claims wherein the oil is a petroleum fuel oil fraction having a viscosity of not more than 1500 mm²/sec at 37.8°C.

8. A method according to claim 6 wherein the oil is a petroleum fuel oil fraction having a viscosity of not more than 850 mm²/sec at 37.8°C.

9. A method according to any of the preceding claims wherein the tumbling ball mill is operated with the contents under an inert gas atmosphere.

10. A method according to any of the preceding claims wherein grinding is carried out at elevated temperature.

11. A method according to any of the preceding claims wherein the mill is rotated at 60 to 95% of its critical speed.

## Revendications

1. Un procédé de préparation d'une dispersion uniforme d'un solide combustible dans une huile, lequel procédé comprend le broyage du solide combustible dans un milieu d'huile combustible jusqu'à ce que la granulométrie moyenne des particules solides soit réduite à une valeur de l'ordre de 1 à 10 µm, la dispersion contenant de 15 à 55% en poids de solide combustible exprimé en tant que pourcentage en poids de l'ensemble de la dispersion, caractérisé en ce que le broyage s'effectue dans un broyeur à boulets culbutants.

2. Un procédé selon la revendication 1, dans lequel la granulométrie moyenne des particules du solide combustible est réduite à une valeur de l'ordre de 2 à 5 µm.

3. Un procédé selon l'une quelconque des revendications précédentes, dans lequel la dispersion contient de 30 à 45% en poids de solide combustible exprimé _{"}n tant que pourcentage en poids de l'en; mble de la dispersion.

4. Un procédé selon l'une quelconque des revendications précédentes, dans lequel le solide friable est du charbon, du charbon raffiné au solvant, du coke de charbon ou du coke de pétrole.

5. Un procédé selon la revendication 4, dans lequel le solide friable est du charbon bitumineux.

6. Un procédé selon l'une quelconque des revendications précédentes, dans lequel le solide combustible est préalablement broyé jusqu'à une granulométrie ne dépassant pas 250 ,um avant le broyage avec l'huile.

7. Un procédé selon l'une quelconque des revendications précédentes, dans lequel l'huile est une fraction d'huile de pétrole ayant une viscosité ne dépassant pas 1500 mm²/sec à 37,8°C.

8. Un proc selon la revendication 6, dans lequel l'huile est une fraction d'huile de pétrole ayant une viscosité ne dépassant pas 850 mm²/sec à 37,8°C.

9. Un procédé selon l'une quelconque des revendications précédentes, dans lequel les produits introduits dans le broyeur à boulets culbutants sont, pendant le fonctionnement, dans une atmosphère de gaz inerte.

10. Un procédé selon l'une quelconque des revendications précédentes, dans lequel le broyage est effectué à température élevée.

11. Un procédé selon l'une quelconque des revendications précédentes, dans lequel le broyeur est entraîné en rotation à une vitesse représentant 60 à 95% de sa vitesse critique.

## Patentansprüche

1. Verfahren zur Herstellung einer gleichmäßigen Dispersion aus einem festen Brennstoff und Öl, wobei der feste Brennstoff in einem Heizölmedium gemahlen wird, bis die mittlere Größe der festen Teilchen auf einen Wert im Bereich von 1 bis 10 ,um vermindert worden ist und die Dispersion 15 bis 55 Gew.- % festen Brennstoff, ausgedrückt als prozentualer Anteil des Gesamtgewichts der Dispersion, enthält, dadurch gekennzeichnet, daß das Mahlen in einer Trommelmühle mit Kugelfüllung stattfindet.

2. Verfahren nach Anspruch 1, dadurch gekennzeichnet, daß die mittlere Größe der festen Teilchen auf einen Wert im Bereich von 2 bis 5 ,um vermindert wird.

3. Verfahren nach einem der vorhergehenden Ansprüche, dadurch gekennzeichnet, daß die Dispersion 30 bis 45 Gew.-% festen Brennstoff, ausgedrückt als prozentualer Anteil des Gesamtegewichts der Dispersion, enthält.

4. Verfahren nach einem der vorhergehenden Ansprüche dadurch gekennzeichnet, daß der zerreibbare Feststoff Kohle, mit Lösungsmittel raffinierte Kohle, Steinkohlenkoks oder Petrolkoks ist.

5. Verfahren nach Anspruch 4, durch gekennzeichnet, daß der zerreibbare Feststoff bituminöse Kohle ist.

6. Verfahren nach einem der vorhergehenden Ansprüche, dadurch gekennzeichnet, daß der feste Brennstoff vor dem Mahlen in dem Ölmedium auf eine Teilchengröße von nicht mehr als 250 um vorgemahlen wird.

7. Verfahren nach einem der vorhergehenden Ansprüche, dadurch gekennzeichnet, daß das Öl eine auf Erdöl stammende Heizöl-Fraktion mit einer Viskosität von nicht mehr als 1500 mm²/s bei 37,8°C ist.

8. Verfahren nach Anspruch 6, dadurch gekennzeichnet, daß das Öl eine aus Erdöl stammende Heizöl-Fraktion mit einer Viskosität von nicht mehr als 850 mm²/s bei 37,8°C ist.

9. Verfahren nach einem der vorhergehenden Ansprüche, dadurch gekennzeichnet, daß die Trommelmühle mit Kugelfüllung mit Inhalt unter einer Inertgas-Atmosphäre betrieben wird.

10. Verfahren nach einem der vorhergehenden Ansprüche, dadurch gekennzeichnet, daß das Mohlen bei erhöhter Temperatur durchgeführt wird.

11. Verfahren nach einem der vorhergehenden Ansprüche, dadurch gekennzeichnet, daß die Mühle mit 60 bis 95% ihrer kritischen Drehgeschwindigkeit betrieben wird.
